

## UNITED STATES PATENT OFFICE

2,209,354

## POTASH CARTRIDGE FOR OXYGEN RESPIRATORS AND LIFESAVER APPARATUS

Heinz Schmidt and Jan Ježek, Usti nad Labem, Czechoslovakia, assignors to Spolek Pro Chemickou A Hutni Výrobu, Usti nad Labem, Aussig A. E., Czechoslovakia

No Drawing. Application February 23, 1938, Serial No. 192,182. In Czechoslovakia May 8, 1937

1 Claim. (Cl. 252—2.5)

In oxygen respirators and lifesaving apparatus, such as is employed more particularly in mining and in fire fighting, so called potash cartridges are provided which are filled with caustic soda and/or caustic potash and to which falls the task of absorbing the carbon dioxide from the spent respiratory air.

The activity of these fillings keeps up in use for only a short time since the caustic alkali, usually present in granulated or lumpy form, becomes coated with a carbonate crust after a short time, which prevents the respiration of air to be regenerated gaining access to the still unspent caustic alkali. This means only incomplete utilisation of the filling and premature passage of insufficiently regenerated respiratory air.

This drawback is met according to the present invention, and the life of the cartridges is substantially increased, by adding to the caustic alkalies, metals, like zinc, aluminium, cadmium and so forth, or compounds thereof alone or in admixture with one another, and preferably in powder form. It has been found that with such additions the caustic alkali is caused to swell up during use, which has the result that always fresh, still uncarbonated, portions of the caustic alkali can act on the respiratory air to be regenerated. Quite a few percent, for example

1-2%, of such additions suffice to attain the desired effect.

*Example*

A hot liquid caustic soda melt is mixed with 2% of its weight of solid aluminium sulphate and the melt homogenised whilst stirring until the sulphate is completely dissolved. The mass is thereupon allowed to set and is granulated in known way. Instead of aluminium sulphate, metallic aluminium or other metals, such as zinc, lead, cadmium and so forth, or compounds thereof, may also be used, alone or in admixture with one another.

As filling for potash cartridges the masses obtained in this way possess on an average a resistance time which is about 50% higher than that of products prepared from usual caustic soda melts.

## What we claim is:

A method of preparing caustic alkali for cartridges for use in respirators and life saving apparatus, consisting in dissolving in a hot liquid caustic alkali bath 2% of its weight of aluminium sulphate, allowing the mass to set, and granulating the set mass.

HEINZ SCHMIDT.

JAN JEŽEK.